# EUROPEAN PATENT SPECIFICATION

(11) **EP 3 561 126 B1**
(45) Date of publication and mention of the grant of the patent: **30.08.2023**
(21) Application number: 17885245.5
(22) Date of filing: 21.12.2017
(51) Int. Cl.: C22C 38/42, C22C 38/44, C22C 38/00, C22C 38/04, C22C 38/58, C21D 8/02, C21D 9/46, C22C 38/02, C22C 38/06

(54) **STEEL MATERIAL HAVING EXCELLENT CORROSION RESISTANCE IN DEW CONDENSATION ENVIRONMENT CONTAINING SULFIDE AND METHOD FOR PRODUCING SAME**
STAHLMATERIAL MIT HERVORRAGENDER KORROSIONSBESTÄNDIGKEIT IN EINER BETAUUNGSUMGEBUNG MIT SCHWEFELWASSERSTOFF UND VERFAHREN ZUR HERSTELLUNG DAVON
MATÉRIAU EN ACIER AYANT UNE EXCELLENTE RÉSISTANCE À LA CORROSION DANS UN ENVIRONNEMENT DE CONDENSATION DE ROSÉE CONTENANT DU SULFURE ET SON PROCÉDÉ DE PRODUCTION

(30) Priority: 22.12.2016 KR 20160177202
(43) Date of publication of application: 30.10.2019
(73) Proprietor: POSCO Co., Ltd, Pohang-si, Gyeongsangbuk-do 37859 (KR)
(72) Inventor: PARK, Jin-Ho, Pohang-si, Gyeongsangbuk-do 37877 (KR); UM, Kyung-Keun, Pohang-si, Gyeongsangbuk-do 37877 (KR)
(74) Representative: Potter Clarkson
(86) International application number: PCT/KR2017/015294
(87) International publication number: WO 2018/117715

(56) References cited:
- JP-A- H07 188 838
- JP-A- S53 115 611
- JP-A- 2002 173 736
- JP-A- 2010 222 701
- JP-A- 2014 201 759
- KR-A- 20100 067 510
- KR-A- 20100 067 510
- KR-A- 20160 085 311
- KR-A- 20160 085 311
- KR-A- 20160 099 063

## Description

### [Technical Field]

The present invention relates to a steel material, having excellent corrosion resistance for use in an oil tanker, a crude oil tank, and the like, and particularly, to a steel material having excellent corrosion resistance in a dew condensation environment containing a sulfide gas and a method for producing the steel material.

### [Background Art]

Among various steels for use in ships, a steel material for use in a crude oil tank for an oil tanker may suffer from significantly serious corrosion damage due to an internal environment of the crude oil tank. In the crude oil tank, various types of corrosion occur due to volatile components in crude, or inert gas, sent into the tank to achieve explosion proofing of mixed seawater, salt in oilfield brine or dew condensation, caused by an internal temperature difference, and the like. Additionally, a corrosion rate is significantly higher than a corrosion rate in a typical brine environment.

In a top plate of a crude tank, hydrogen sulfide gas, evaporated from crude, and gas such as CO₂, SO₂, O₂ or the like in inert gas, introduced to achieve explosion proofing, may react with dew condensation, formed on a surface of a steel material by a temperature difference, to contain a large amount of hydrogen sulfide and sulfur dioxide components. Accordingly, corrosion occurs. Corrosion caused by the dew condensation, i.e. condensed water, is similar to atmospheric corrosion of atmospheric corrosion resistant steel because of the corrosion at the thin water film, and moisture is periodically and repeatedly condensed and dried due to a daily temperature range. For this reason the corrosion, caused by condensed water, may be separately classified as dew point corrosion.

During daytime, dew condensation does not occur on the deckhead of a crude oil transport ship, running while loaded with crude oil, because an internal temperature of the deckhead rises to about 50°C. During nighttime, evaporated moisture forms on a lower portion of the deckhead because the internal temperature of the deckhead drops to about 25°C. In the case of a 300,000 ton crude oil transport ship, up to 30 tons of water may condense on an upper portion of a deckhead to cause corrosion. Therefore corrosion, caused by the condensed water, is not negligible.

In addition carbon dioxide and sulfur dioxide, which are incombustible gases, are injected into an empty space in a tank of a crude oil transport ship to prevent the explosion of a hull. Such gases are dissolved in moisture, together with sulfur and hydrogen sulfide, already contained in crude oil, to form an atmosphere proximate to corrosion caused by acidic condensed water when dew condensation occurs. Generally, as acidity is increased, an amount of H⁺ ions, participating in a corrosion reaction, is increased. Therefore, a corrosion rate may be further increased.

Patent Document 1 has been proposed to improve corrosion resistance of a steel material for a ship. However, since a steel material for a ship of Patent Document 1 was designed without consideration of corrosion caused by hydrogen sulfide when crude oil contains the hydrogen sulfide, the steel material for ship is insufficient to be used in an actual crude oil tank.
(Patent Documents 1) Japanese Patent Publication Laid-Open 2000-017381. Steels are disclosed in JP S53115611 A and JP H07188838 A. Other solutions are disclosed in JP 2010-222701 A, KR 2016-0085311 A, KR 2010-0067510 A.

### [Disclosure]

### [Technical Problem]

The present invention is to provide a steel material which may optimize steel components and may identify a relationship between components to secure improved corrosion resistance, even in a dew condensation environment including sulfides; and a method for producing the steel material.

### [Technical Solution]

The steel material according to the invention is defined in the independent claim 1. The method for producing a steel material according to the invention is defined in the independent claim 3. The preferred embodiments are defined in the dependent claims.

### [Advantageous Effects]

As set forth above, according to the present invention steel components are optimized to satisfy a sensitivity index of sulfide dew point corrosion. Thus, resistance against the sulfide dew point corrosion may be improved.

### [Description of Drawings]

FIG. 1 illustrates a test apparatus for simulating a sulfide dew condensation test in the present disclosure.
FIG. 2 is an image illustrating a result of a sulfide dew point corrosion test performed for 100 days according to an example embodiment in the present invention. Steels 3 and 4 refer to the reference steels 3 and 4.

### [Best Mode for Invention]

Hereinafter, the present invention will be described in detail.

The present inventors have conducted researches to address the above-described issues of the related art. The inventors found that in order to improve resistance against corrosion in a dew condensation environment containing sulfide gas, a composition of each component needs to be appropriately controlled, as set forth below. In addition, the inventors found that that relationships between components such as Ca, S, Cr, Mo, Ni, Mn, and the like, affecting sensitivity of dew point corrosion, needs to be appropriately controlled. For these reasons, the inventors conceived the present invention.

First, an alloy composition range of a steel material according to the present disclosure will be described in detail. The steel material comprises, by weight percent (wt%), 0.02 to 0.2% of carbon (C), 0.1 to 1.0% of silicon (Si), 0.2 to 2.0% of manganese (Mn), 0.03% or less of phosphorus (P), 0.03% or less of sulfur (S), 0.05 to 0.5% of copper (Cu), 0.05 to 0.5% of nickel (Ni), 0.02 to 0.5% of molybdenum (Mo), 0.1% or less of aluminum (Al), 0.05 to 0.5% of chromium (Cr), 0.001 to 0.01% of calcium (Ca), and a balance of iron (Fe) and inevitable impurities.

### Carbon (C): 0.02 to 0.2 wt%

Carbon (C) is an element added to improve strength. When a content of carbon (C) is increased, hardenability may be increased to improve strength. However, as the amount of added carbon is increased, general corrosion resistance is reduced. And since precipitation of carbide or the like is promoted, localized corrosion resistance is also affected. The content of carbon (C) should be decreased to improve the general corrosion resistance and the localized corrosion resistance. However, when the content of carbon (C) is less than 0.02 wt%, it is difficult to secure strength. When carbon (C) is more than 0.2 wt%, weldability is deteriorated to be inappropriate for, in detail, steel for welded structure. Therefore, carbon (C) has a range, in detail, from 0.02 to 0.2 wt%. Under a viewpoint of corrosion resistance, the content of carbon (C) may be set to, in detail, be 0.16 wt% or less and may be set to, in further detail, 0.14 wt% or less to improve casting cracking and to reduce a carbon equivalent.

### Silicon (Si): 0.1 to 1.0 wt%

Silicon (Si) needs to be present in amount of 0.1 wt% or more to serve as a deoxidizer and to serve to increase strength of steel. In addition, since silicon (Si) contributes to improvement in general corrosion resistance, it is advantageous to increase the content of silicon (Si). However, when the content of silicon (Si) is greater than 1.0 wt%, toughness and weldability are deteriorated. And since it is difficult to detach a scale during rolling, the scale causes a surface defect. Therefore, the content of silicon (Si) is limited to, in detail, 0.1 to 1.0 wt%. In further detail, silicon (Si) is added in an amount of 0.2 wt% or more to improve corrosion resistance.

### Manganese (Mn): 0.2 to 2.0 wt%

Manganese (Mn) is an element effect in increasing the strength without reducing toughness. However, when an excessive amount of manganese (MN) is added, an electrochemical reaction rate of a steel surface may be increased during a corrosion reaction to reduce corrosion resistance. When manganese (Mn) is added in an amount of less than 0.2 wt%, it is difficult to secure durability of a structural steel. When the content of manganese (Mn) is increased, hardenability is increased to improve strength. However, when manganese (Mn) is added in an amount greater than 2.0 wt%, weldability and corrosion resistance are reduced. Therefore, the content of manganese (Mn) is set to be, in detail, 0.2 to 2.0 wt%.

### Phosphorus (P): 0.03 wt% or less

Phosphorus (P) is an impurity element. When the phosphorous (P) is added in an amount greater than 0.03 wt%, weldability is significantly reduced and toughness is deteriorated. Therefore, the content of phosphorous (P) is limited to, in detail, 0.03 wt% or less.

### Sulfur (S): 0.03 wt% or less

Sulfur (S) is also an impurity element. When the content of sulfur (S) is greater than 0.03 wt%, ductility, impact toughness, and weldability of steel are deteriorated. Accordingly, the content of sulfur (S) is limited to, in detail, 0.03 wt% or less. Sulfur (S) is apt to react with manganese (Mn) to form an elongated inclusion like manganese sulfide (MnS), and voids, formed on both ends of the elongated inclusion, may be a starting point of localized corrosion. Therefore, the content of sulfur (S) is limited to, in further detail, 0.01 wt% or less.

### Copper (Cu): 0.05 to 0.5 wt%

When copper (Cu) is contained in an amount of 0.05 wt% or more together with nickel (Ni), exudation of iron (Fe) is delayed, which is effective in improving general corrosion resistance and localized corrosion resistance. However, when the amount of copper (Cu) is greater than 0.5 wt%, copper (Cu) in a liquid state melts into a grain boundary during production of a slab. Thus, cracking occurs during hot working, which is called "hot shortness" phenomenon. Therefore, the content of copper (Cu) is set to, in detail, be 0.05 to 0.5 wt%. Since surface cracking, occurring during production of the slab, interact with the contents of carbon (C), nickel (Ni), and manganese (Mn), a frequency of occurrence of the surface cracking may vary, depending on the content of each element, but the content of copper (Cu) is set to, in further detail, be 0.5 wt% or less.

### Nickel (Ni): 0.05 to 0.5 wt%

Similarly to the case of copper (Cu), when nickel (Ni) is contained in an amount of 0.05 wt% or more, it is effective in improving general corrosion resistance and localized corrosion resistance. In addition, when nickel (Ni) is added together with copper (Cu), nickel (Ni) reacts with copper (Cu) in such a manner that formation of a copper (Cu) phase is suppressed to prevent hot shortness from occurring. Nickel (Ni) is also an element effective in improving toughness of a base material. However, since nickel (Ni) is an expensive element, the addition of nickel (Ni) in an amount of 0.5 wt% or more is disadvantageous in terms of economical efficiency and weldability. Therefore, the content of nickel (Ni) is set to, in detail, be 0.05 to 0.5 wt%.

Since an influence of nickel (Ni) on improvement of corrosion resistance is not higher than an influence of copper (Cu), the content of nickel (Ni) is greater than the content of copper (Cu), in detail, 1.5 times or less the content of copper (Cu) to suppress surface cracking caused by addition of copper (Cu), rather than containing a great amount of nickel (Ni) to improve corrosion resistance. The content of nickel (Ni) is limited to, in further detail, 0.3 wt% or less.

### Molybdenum (Mo): 0.02 to 0.5 wt%

Molybdenum (Mo) is an element contributing to improvement of corrosion resistance and strength and should be added in an amount of 0.02 wt% or more to achieve such an effect. However, molybdenum (Mo) should be dissolved in steel to improve corrosion resistance. For example, the dissolved molybdenum (Mo) improves the corrosion resistance to the condensed water containing hydrogen sulfide. However, molybdenum (Mo), contained in an amount greater than a dissolution limit, may reacts with sulfur (S) in such a manner Mo₂S is formed to reduce corrosion resistance. Therefore, when an excessive amount of molybdenum (Mo) is added, corrosion resistance against condensed water, containing hydrogen sulfide, may be reduced. Hence, an upper limit thereof is, in detail, 0.5 wt%. In addition, a precipitate of molybdenum (Mo) serves to improve strength, but coarsely precipitated molybdenum (Mo) may cause localized corrosion of the steel. Therefore, molybdenum (Mo) is added in an amount of, in further detail, 0.1 wt% or less.

### Aluminum (Al): 0.1 wt% or less

Aluminum (Al) is an element, added for deoxidation, and reacts with nitrogen (N) in the steel in such a manner that an aluminum nitride (AlN) is formed and austenite grains are refined to improve toughness. However, when aluminum(Al) is contained in an amount greater than 0.1 wt%, an inclusion is formed in a coarse oxide during a steelmaking process and a stretched inclusion, crushed and elongated during rolling, is formed according to aluminum oxide-based characteristics. Since the formation of such an elongated inclusion promotes the formation of a void around the inclusion and such a void serves as a starting point for localized corrosion, the elongated inclusion serves to reduce the localized corrosion resistance. Therefore, the content of aluminum (Al) is set to, in detail, be 0.1 wt% or less. Since deoxidation effect may be obtained by another deoxidizing element such as silicon (Si) or the like even when aluminum (Al) is added, a lower limit of aluminum (Al) is not limited. However, in detail, at least 0.001 wt% or more of aluminum (Al) may be added to expect a deoxidation effect achieved by aluminum (Al).

### Chromium (Cr): 0.05 to 0.5 wt%

Chromium (Cr) is an element which increases the corrosion resistance by forming a chrome-containing oxide layer on a surface of the steel in a corrosive environment. Chromium (Cr) should be contained in an amount of 0.05 wt% or more to exhibit a corrosion resistance effect depending on addition of chromium (Cr). However, when chromium (Cr) is contained in an amount greater than 0.5 wt%, toughness and weldability are adversely affected. Therefore, the content of chromium (Cr) is set to, in detail, be 0.05 to 0.5 wt%.

### Calcium (Ca): 0.001 to 0.01 wt%

Calcium (Ca) reacts with aluminum (Al), silicon (Si), and oxygen (O) in a molten steel to form a composite oxide and then reacts with sulfur (S) to form calcium sulfide (CaS). Such a calcium sulfide (CaS) inclusion is dissolved in water in a dew condensation environment to increase pH of the surface of the steel. Thus, formation of a stable phase is promoted under suppress of an electrochemical reaction of the steel to improve corrosion resistance characteristics. To improve the corrosion resistance, calcium (Ca) should be added in an amount of at least 0.001 wt%. However, when the content of calcium (Ca) is greater than 0.01 wt%, refractories may be melted during a steelmaking process. Therefore, the content of Ca is set to, in detail, be 0.001 to 0.01 wt%. Additionally, calcium (Ca) is added in an amount of, in further detail, 0.002 wt% or more to secure a sulfide dew point corrosion sensitivity index.

In addition to the above components, the balance is iron (Fe) and inevitable impurities.

In the steel material of the present invention, the sulfide condensation corrosion sensitivity index, defined as Relational Expression 1, satisfies, in detail, 1.78 to 2.25.

### Relational Expression 1

$\begin{matrix}Sensitivity Index of Sulfide Dew point corrosion = 0.4 Ca / S \\ + 5 Cr + 6Mo + 2 Cu + Ni - 0.5 Mn\end{matrix}$ (where Ca, S, Cr, Mo, Cu, Ni, and Mn denote contents (wt%) of corresponding elements).

The above Ca, Cr, Mo, Cu, Ni, and Mn are components affecting a corrosion resistance effect in a sulfide dew condensation environment depending on amounts of addition thereof. An influence of each of these components on the corrosion resistance was quantitatively derived, and a relationship between the components was expressed by Relational Expression 1. When the sensitivity index of sulfide dew point corrosion, defined as Relational Expression 1, is 1.7 to 2.5, improved corrosion resistance may be secured in a corresponding environment. According to the invention, the sensitivity index of sulfide dew point corrosion, defined as Relational Expression 1, is 1.78 to 2.25.

The steel of the present invention, having the advantageous composition, may be easily produced using knowledge in the art by a person of ordinary skill in the art without excessively repeated tests. A method for producing the steel material is proposed in the present invention .

The method for producing a steel material according to the present invention is a method for producing a steel material through conventional hot rolling and cooling, and is characterized in that the cooling is performed at a cooling rate of 10°C/sec or higher in such a manner that cooling starting temperature is Ar3 temperature or higher and cooling stop temperature ranges from (Ae1-30°C) to 600°C. Hereinafter, cooling conditions of the present disclosure will be described.

### Cooling Section: cooled from Ar3 temperature or higher to (Ae1-30°C) - 600°C

According to a result of tests performed by the present inventors, when molybdenum (Mo), added to achieve the advantageous effect, forms a great amount of precipitate, the added molybdenum (Mo) has an adverse influence on general corrosion, localized corrosion, or the like. Meanwhile, when an excessive amount of molybdenum (Mo) is dissolved, molybdenum (Mo) has an adverse influence on corrosion resistance in an environment containing hydrogen sulfide. Therefore, it is necessary to appropriately control a ratio of molybdenum (Mo), forming the precipitate, and the dissolved molybdenum (Mo). Since molybdenum (Mo) tends to form precipitates at temperature between 700 and 550°C, a portion of the section needs to be rapidly cooled to prevent that molybdenum (Mo) forms a precipitate and the other portions of the section need to be slowly cooled to prevent that molybdenum (Mo) is excessively dissolved.

When cooling is started at temperature lower than the Ar3 temperature, copper (Cu) is segregated to pearlite to accelerate corrosion caused by a galvanic pair of the pearlite and ferrite. Accordingly, the cooling needs to be started at temperature, higher than or equal to the Ar3 temperature, and needs to be performed to a temperature of (Ae1-30°C) or lower at which precipitates such as molybdenum (Mo) are appropriately formed without forming pearlite . When the cooling is performed to significantly low temperature, molybdenum (Mo) is not appropriately precipitated and is excessively dissolved. Therefore, molybdenum (Mo) may bond to sulfur (S) at a condensed water atmosphere, containing hydrogen sulfide, to form MozS and may deteriorate corrosion resistance of the steel material. As a result, the cooling needs to be finished at temperature of 600°C or higher.

### Cooling Rate: 10°C/s or higher

Since time, taken to pass through a temperature range in which a precipitate of molybdenum (Mo) is easily formed, is increased when the cooling rate is low, the precipitate may be excessively formed. Therefore, the cooling rate needs to be 10°C/s or higher. Even if the cooling rate is high, there is no problem in achieving objects of the present disclosure. Accordingly, it is unnecessary to determine an upper limit of the cooling rate. However, since there may be a limitation in capability of cooling equipment, the upper limit may be determined to be 50°C/s in consideration of the limitation in capability to apply a significantly high cooling rate.

### [Mode for Invention]

Hereinafter, an example embodiment in the present invention will be described in detail. However, the present invention is not limited to the example embodiment described herein.

### (Embodiment)

A steel slab was produced using continuous casting after preparing molten steel having a composition (weight percent (wt%), the balance including iron (Fe) and inevitable impurities) listed in Table 1. The produced steel slab was hot-rolled under normal conditions and then cooled under conditions in Table 2.

**Table 1**

| Steel No. | C | Si | Mn | P | S | Ni | Mo | Al | Cu | Cr | Ca |
|---|---|---|---|---|---|---|---|---|---|---|---|
| IS 1 | 0.06 | 0.45 | 0.9 | 0.015 | 0.003 | 0.35 | 0.05 | 0.025 | 0.25 | 0.2 | 0.004 |
| IS 2 | 0.08 | 0.61 | 1.1 | 0.02 | 0.002 | 0.26 | 0.03 | 0.03 | 0.22 | 0.15 | 0.004 |
| RS 3 | 0.09 | 0.81 | 1.2 | 0.02 | 0.004 | 0.4 | 0.12 | 0.029 | 0.1 | 0.09 | 0.008 |
| RS 4 | 0.04 | 0.75 | 0.9 | 0.019 | 0.003 | 0.31 | 0.04 | 0.034 | 0.14 | 0.12 | 0.007 |
| IS 5 | 0.12 | 0.51 | 0.8 | 0.012 | 0.003 | 0.4 | 0.05 | 0.031 | 0.3 | 0.11 | 0.006 |
| IS 6 | 0.16 | 0.31 | 1.4 | 0.022 | 0.006 | 0.29 | 0.03 | 0.027 | 0.19 | 0.3 | 0.002 |
| IS 7 | 0.15 | 0.5 | 0.7 | 0.011 | 0.005 | 0.24 | 0.06 | 0.021 | 0.21 | 0.25 | 0.003 |
| CS 1 | 0.07 | 0.45 | 0.9 | 0.012 | 0.004 | 0.21 | 0 | 0.035 | 0.15 | 0.15 | 0.002 |
| CS 2 | 0.11 | 0.52 | 1.2 | 0.018 | 0.004 | 0.22 | 0.02 | 0.031 | 0.16 | 0.21 | 0.001 |
| CS 3 | 0.09 | 0.49 | 0.8 | 0.017 | 0.004 | 0.16 | 0.04 | 0.029 | 0.12 | 0.2 | 0.003 |
| CS 4 | 0.1 | 0.51 | 1.1 | 0.016 | 0.005 | 0.19 | 0.05 | 0.034 | 0.14 | 0.25 | 0.001 |
| CS 5 | 0.06 | 0.68 | 1.5 | 0.015 | 0.003 | 0.45 | 0.02 | 0.036 | 0 | 0.2 | 0.004 |
| CS 6 | 0.1 | 0.56 | 1.2 | 0.018 | 0.005 | 0.4 | 0.05 | 0.036 | 0.3 | 0 | 0.006 |
| CS 7 | 0.1 | 0.6 | 1.3 | 0.018 | 0.008 | 0.15 | 0.2 | 0.029 | 0.1 | 0.35 | 0.001 |
| CS 8 | 0.08 | 0.55 | 1.2 | 0.013 | 0.007 | 0.21 | 0.17 | 0.027 | 0.12 | 0.31 | 0.002 |

| | | | | | | | | | | | |
|---|---|---|---|---|---|---|---|---|---|---|---|
| *IS: Inventive Steel ^{∗}RS:Reference Steel *CS: Comparative Steel | | | | | | | | | | | |

**Table 2**

| Steel No. | Ar3 (°C) | Cooling Starting Temperature (°C) | Cooling Ending Temperature (°C) | Cooling Rate (°C/s) |
|---|---|---|---|---|
| IS 1 | 794 | 815 | 658 | 17.3 |
| IS 2 | 780 | 812 | 634 | 19.7 |
| RS 3 | 757 | 805 | 647 | 17.5 |
| RS 4 | 807 | 829 | 622 | 21.8 |
| IS 5 | 781 | 819 | 634 | 20.1 |
| IS 6 | 728 | 778 | 651 | 14.6 |
| IS 7 | 788 | 809 | 647 | 17.5 |
| CS 1 | 806 | 820 | 644 | 19.2 |
| CS 2 | 766 | 791 | 618 | 18.5 |
| CS 3 | 807 | 834 | 634 | 20.9 |
| CS 4 | 776 | 807 | 627 | 19.8 |
| CS 5 | 748 | 798 | 613 | 20.1 |
| CS 6 | 757 | 789 | 618 | 18.5 |
| CS 7 | 750 | 781 | 616 | 17.9 |
| CS 8 | 763 | 777 | 620 | 17.1 |

| | | | | |
|---|---|---|---|---|
| *IS: Inventive Steel ^{∗}RS:Reference Steel *CS: Comparative Steel | | | | |

As can be seen from the Table 1, inventive steels refer to steel sheets having compositions satisfying a composition range defined in the present invention . However, comparative steels 1, 5, and 6 illustrate a case in which essential additive elements, selected in the present disclosure, such as Mo, Cu, and Cr are not added. Comparative steels 2, 3, 4, 7, and 8 illustrate a case in which essential elements are added but the sensitivity index of sulfide dew point corrosion, expressed as Relational Expression 1, does not satisfy a required range because the sensitivity index is less than 1.7 or more than 2.5, as described later. Such components of the comparative steels are significantly reduced in corrosion resistance than those of the inventive steels. Accordingly, since corrosion of the steel material cannot be prevented in the sulfide dew point corrosion environment, the corrosion resistance may be reduced and a replacement cycle may be increased. The reference steels do not satisfy the claimed Relational Expression 1.

Table 3 below lists measurement results of sensitivity indices of sulfide dew point corrosion and corrosion rates of inventive steels and comparative steels. The corrosion rates, listed in Table 3, were results measured by the test apparatus illustrated in FIG. 1. For example, as illustrated in FIG. 1, in order to simulate the sulfide dew condensation environment, an airtight container was filled with distilled water and a corrosive gas such as SO₂, H₂S, CO₂, O₂, or the like was continuously purged into the distilled water. Then a sample, having a size of 60mm × 20mm × 5mm, to measure a corrosion rate was polished with #600 sandpaper and located on top of the airtight container. A cover of the airtight container was provided with a gas inlet, an outlet, and a heating/cooling water circulation system. After being air-tightened, the airtight container was mounted in a thermostat and a temperature cycle of (50°C, 20 hours) → (25°C, 4 hours) was given for 100 days. A gas, introduced into the test apparatus, was a gas simulating the sulfide dew point corrosion environment of an upper deck of the crude oil tank, and has a composition below.
Gas Composition: by volume percent, 5% of O₂ - 15% of CO₂ - 0.011% of SO₂ - 0.055% of H₂S - balance N₂

After a corrosion test for 100 days, a derusting treatment was performed in a corrosion product removal solution. Mass loss of each sample was divided by a surface area of an initial sample. For relative comparison, the corrosion rate of the comparative steel 1 was set to 100, and relative corrosion rates are listed in Table 3.

**Table 3**

| Steel No. | Sensitivity Index of Sulfide Dew point corrosion | Relative Corrosion Rate |
|---|---|---|
| IS 1 | 2.23 | 38 |
| IS 2 | 1.88 | 49 |
| RS 3 | 1.97 | 42 |
| RS 4 | 1.91 | 45 |
| IS 5 | 2.25 | 34 |
| IS 6 | 1.78 | 57 |
| IS 7 | 2.16 | 37 |
| CS 1 | 1.01 | 100 |
| CS 2 | 1.21 | 95 |
| CS 3 | 1.54 | 90 |
| CS 4 | 1.55 | 90 |
| CS 5 | 1.35 | 88 |
| CS 6 | 1.18 | 85 |
| CS 7 | 2.70 | 69 |
| CS 8 | 2.53 | 65 |

| | | |
|---|---|---|
| *IS: Inventive Steel *RS: Reference Steel *CS: Comparative Steel | | |

As can be seen from Table 2, when the corrosion resistance element such as Mo, Cu, Cr, or the like is not added at all or is insufficiently added and the sensitivity index of sulfide dew condensation does not satisfy a range of more than 1.7 to less than 2.3, a relative corrosion rate is at most twice as high as that of the inventive steel. Such a phenomenon occurred in all comparative steels although the degree thereof was slightly different, which is determined to result from the fact that the sensitivity index of sulfide dew condensation of 1.7-2.3 was not satisfied.

FIG. 2 is an image of samples of the inventive steels 1, 2, 5-7, and reference steels 3 and 4 and the comparative steels 1 to 8 observed after a sulfide dew point corrosion test performed for 100 days. As described above, the inventive steels 1, 2, 5-7, and reference steels 3 and 4 in which the sensitivity index of sulfide dew corrosion satisfies the range of 1.7 or more to 2.5 or less of

Relational Expression 1, had a dense structure in which corrosion products had bright colors. In the case of the comparative steels 1 to 8, dark-colored corrosion products are visible to the naked eye.

As described above, as illustrated in Table 3 and FIG. 2, the sensitivity index of sulfide corrosion, should be satisfied to to be between 1.7 and 2.3 to prevent sulfide dew point corrosion. According to the invention, the sensitivity index of sulfide dew point corrosion, defined as Relational Expression 1, is 1.78 to 2.25.

When the sensitivity index is not satisfied, sufficient corrosion resistance is not secured to stably use a steel material in a corresponding environment, and thus life of a corresponding structure may not be secured.

## Claims

1. A steel material, having excellent corrosion resistance in a dew condensation environment containing a sulfide gas, comprising, by weight percent, 0.02 to 0.2% of carbon (C), 0.1 to 1.0% of silicon (Si), 0.2 to 2.0% of manganese (Mn), 0.03% or less of phosphorus (P), 0.03% or less of sulfur (S), 0.05 to 0.5% of copper (Cu), 0.05 to 0.5% of nickel (Ni), 0.02 to 0.5% of molybdenum (Mo), 0.1% or less of aluminum (Al), 0.05 to 0.5% of chromium (Cr), 0.001 to 0.01% of calcium (Ca), and the balance of iron (Fe) and inevitable impurities,
wherein a sensitivity index of sulfide dew point corrosion, given by Relational Expression 1, is 1.78 or more to 2.25 or less: $\begin{matrix}Sensitivity Index of Sulfide Dew \\ point corrosion = 0.4 Ca / S + 5 Cr + 6Mo + 2 Cu + Ni - 0.5 Mn\end{matrix}$
where Ca, S, Cr, Mo, Cu, Ni, and Mn denote contents by weight percent of corresponding elements, and
wherein a content of the Ni is greater than a content of the Cu, and is 1.5 times or less the content of the Cu.

2. The steel material of claim 1, wherein the Ca is 0.002 to 0.01%.

3. A method for producing a steel material, having excellent corrosion resistance in a dew condensation environment containing a sulfide gas, by hot-rolling and cooling a slab comprising, by weight percent, 0.02 to 0.2% of carbon (C), 0.1 to 1.0% of silicon (Si), 0.2 to 2.0% of manganese (Mn), 0.03% or less of phosphorus (P), 0.03% or less of sulfur (S), 0.05 to 0.5% of copper (Cu), 0.05 to 0.5% of nickel (Ni), 0.02 to 0.5% of molybdenum (Mo), 0.1% or less of aluminum (Al), 0.05 to 0.5% of chromium (Cr), 0.001 to 0.01% of calcium (Ca), and the balance of iron (Fe) and inevitable impurities,
wherein a sensitivity index of sulfide dew point corrosion, given by Relational Expression 1, is 1.78 or more to 2.25 or less: $\begin{matrix}Sensitivity Index of Sulfide Dew \\ point corrosion = 0 .4Ca / S + 5 Cr + 6 Mo + 2 Cu + Ni - 0.5 Mn\end{matrix}$
where Ca, S, Cr, Mo, Cu, Ni, and Mn denote contents (wt%) of corresponding elements, and
wherein the cooling is performed at a cooling rate of 10°C/s or higher between cooling start temperature, higher than or equal to Ar3 temperature, and cooling stop temperature of (Ae1-30°C) to 600°C, and
wherein a content of the Ni is greater than a content of the Cu, and is 1.5 times or less the content of the Cu.

4. The method of claim 3, wherein the Ca is 0.002 to 0.01%.

## Patentansprüche

1. Stahlwerkstoff mit ausgezeichneter Korrosionsbeständigkeit in einer Taukondensationsumgebung, die ein Sulfidgas enthält, umfassend, in Gewichtsprozent, 0,02 bis 0,2 % Kohlenstoff (C), 0,1 bis 1,0 % Silizium (Si), 0,2 bis 2,0 % Mangan (Mn), 0,03 % oder weniger Phosphor (P), 0,03 % oder weniger Schwefel (S), 0,05 bis 0,5 % Kupfer (Cu), 0,05 bis 0,5 % Nickel (Ni), 0,02 bis 0,5 % Molybdän (Mo), 0,1 % oder weniger Aluminium (Al), 0,05 bis 0,5 % Chrom (Cr), 0,001 bis 0,01 % Kalzium (Ca) und als Rest Eisen (Fe) und unvermeidliche Verunreinigungen,
wobei ein Empfindlichkeitsindex der Sulfid-Taupunktkorrosion, angegeben durch den Vergleichsausdruck 1, 1,78 oder mehr bis 2,25 oder weniger beträgt:
Vergleichsausdruck 1: Empfindlichkeitsindex der Sulfid-Taupunktkorrosion = 0,4Ca/S + 5Cr + 6Mo + 2Cu + Ni - 0,5Mn
wobei Ca, S, Cr, Mo, Cu, Ni und Mn die Gehalte in Gewichtsprozent der entsprechenden Elemente bezeichnen,
und wobei ein Gehalt an Ni größer ist als ein Gehalt an Cu und das 1,5-fache oder weniger des Gehalts an Cu beträgt.

2. Stahlwerkstoff nach Anspruch 1, wobei der Ca-Gehalt 0,002 bis 0,01 % beträgt.

3. Verfahren zur Herstellung von Stahlwerkstoff mit ausgezeichneter Korrosionsbeständigkeit in einer Taukondensationsumgebung, die ein Sulfidgas enthält, durch Warmwalzen und Abkühlen einer Bramme, umfassend, in Gewichtsprozent, 0,02 bis 0,2 % Kohlenstoff (C), 0,1 bis 1,0 % Silizium (Si), 0,2 bis 2,0 % Mangan (Mn), 0,03 % oder weniger Phosphor (P), 0,03 % oder weniger Schwefel (S), 0,05 bis 0,5 % Kupfer (Cu), 0,05 bis 0,5 % Nickel (Ni), 0,02 bis 0,5 % Molybdän (Mo), 0,1 % oder weniger Aluminium (Al), 0,05 bis 0,5 % Chrom (Cr), 0,001 bis 0,01 % Kalzium (Ca) und als Rest Eisen (Fe) und unvermeidliche Verunreinigungen,
wobei ein Empfindlichkeitsindex der Sulfid-Taupunktkorrosion, angegeben durch den Vergleichsausdruck 1, 1,78 oder mehr bis 2,25 oder weniger beträgt:
Vergleichsausdruck 1: Empfindlichkeitsindex der Sulfid-Taupunktkorrosion = 0,4Ca/S + 5Cr + 6Mo + 2Cu + Ni - 0,5Mn
wobei Ca, S, Cr, Mo, Cu, Ni und Mn die Gehalte (Gew.-%) der entsprechenden Elemente bezeichnen, und
wobei die Abkühlung mit einer Abkühlungsrate von 10°C/s oder mehr zwischen der Abkühlungsstarttemperatur, die höher als oder gleich der Ar3-Temperatur ist, und der Abkühlungsstopptemperatur von (Ael-30°C) bis 600°C durchgeführt wird, und
wobei der Ni-Gehalt größer ist als der Cu-Gehalt und das 1,5-fache oder weniger des Cu-Gehalts beträgt.

4. Verfahren nach Anspruch 3, wobei der Ca-Gehalt 0,002 bis 0,01 % beträgt.

## Revendications

1. Matériau en acier, ayant une excellente résistance à la corrosion dans un environnement de condensation de rosée contenant un sulfure gazeux, comprenant, en pourcentage de poids, 0,02 à 0,2 % de carbone (C), 0,1 à 1,0 % de silicium (Si), 0,2 à 2,0 % de manganèse (Mn), 0,03 % ou moins de phosphore (P), 0,03 % ou moins de soufre (S), 0,05 à 0,5 % de cuivre (Cu), 0,05 à 0,5 % de nickel (Ni), 0,02 à 0,5 % de molybdène (Mo), 0,1 % ou moins d'aluminium (Al), 0,05 à 0,5 % de chrome (Cr), 0,001 à 0,01 % de calcium (Ca), et le reste de fer (Fe) et d'impuretés inévitables,
dans lequel un indice de sensibilité de la corrosion au point de rosée du sulfure, donné par l'expression relationnelle 1, est de 1,78 ou plus à 2,25 ou moins : $\begin{matrix}Indice de sensibilité \\ de la corrosion au point de rosée de sulfure = 0,4 Ca / S \\ + 5 CR + 6 Mo + 2 Cu + Ni - 0,5 Mn\end{matrix}$
où Ca, S, Cr, Mo, Cu, Ni et Mn désignent des teneurs en pourcentage de poids d'éléments correspondants, et
dans lequel une teneur en Ni est supérieure à une teneur en Cu, et est égale ou inférieure à 1,5 fois la teneur en Cu.

2. Matériau en acier selon la revendication 1, dans lequel le Ca est de 0,002 à 0,01 %.

3. Procédé de production d'un matériau en acier, ayant une excellente résistance à la corrosion dans un environnement de condensation de rosée contenant un sulfure gazeux, par laminage à chaud et refroidissement d'une brame comprenant, en pourcentage de poids, 0,02 à 0,2 % de carbone (C), 0,1 à 1,0 % de silicium (Si), 0,2 à 2,0 % de manganèse (Mn), 0,03 % ou moins de phosphore (P), 0,03 % ou moins de soufre (S), 0,05 à 0,5 % de cuivre (Cu), 0,05 à 0,5 % de nickel (Ni), 0,02 à 0,5 % de molybdène (Mo), 0,1 % ou moins d'aluminium (Al), 0,05 à 0,5 % de chrome (Cr), 0,001 à 0,01 % de calcium (Ca), et le reste de fer (Fe) et d'impuretés inévitables,
dans lequel un indice de sensibilité de la corrosion au point de rosée de sulfure, donné par l'expression relationnelle 1, est de 1,78 ou plus à 2,25 ou moins : $\begin{matrix}Indice de sensibilité \\ de la corrosion au point de rosée de sulfure = 0,4 Ca / S \\ + 5 Cr + 6 Mo + 2 Cu + Ni - 0,5 Mn\end{matrix}$
où Ca, S, Cr, Mo, Cu, Ni et Mn désignent les teneurs (en pourcentage de poids) des éléments correspondants, et
dans lequel le refroidissement est effectué à une vitesse de refroidissement de 10 °C/s ou plus entre la température de début de refroidissement, supérieure ou égale à la température Ar3, et la température d'arrêt de refroidissement de (Ael-30 °C) à 600 °C, et
dans lequel une teneur en Ni est supérieure à une teneur en Cu, et est égale ou inférieure à 1,5 fois la teneur en Cu.

4. Procédé selon la revendication 3, dans lequel le Ca est de 0,002 à 0,01 %.
